

## UNITED STATES PATENT OFFICE

2,099,120

## FLOTATION PROCESS

James Emory Kirby and James Herbert Werntz,  
Wilmington, Del., assignors to E. I. du Pont de  
Nemours & Company, Wilmington, Del., a cor-  
poration of Delaware

No Drawing. Application October 15, 1936,  
Serial No. 105,676

10 Claims. (Cl. 209—166)

This invention relates to a method of separating the valuable mineral constituents of naturally occurring ores from the worthless or gangue materials. More particularly, it relates to an improved froth flotation method for separating and concentrating the desired mineral constituents of natural ores. Still more particularly, it relates to the use of certain water-soluble salts of half esters of organic di-basic acids in an improved froth flotation process especially applicable to the group of materials comprising the non-sulfide ores and coal.

This invention has as its object the development of an improved froth flotation method for the concentration of ores and minerals, particularly those of the class comprising non-sulfidic ores and coal. A further object is the development of a froth flotation method for treating non-sulfide ores and coal having better selectivity than those heretofore known. Still another object is to provide a class of collecting and frothing agents for use in the flotation of non-sulfidic ores and coal, whose collecting strength, selectivity, and frothing power can be controlled by a suitable choice of constituents used in preparing the flotation reagent. Another object is to provide a reagent for use in coal flotation which gives froths of better characteristics than those previously used. Further objects will appear hereinafter.

These objects are accomplished by utilizing as a flotation reagent a water-soluble salt of an organic di-carboxylic acid having one carboxyl group esterified by an alcohol chosen from the class comprised of straight chain aliphatic primary alcohols having from 8 to 18 carbon atoms and alicyclic alcohols derived by carboxylic reduction from naphthenic acids and natural resin acids.

In carrying out the process of this invention, a slurry of ground ore or coal and water (known as an ore or coal pulp) is treated with a small amount, usually from 0.05 pound to 2-3 pounds per ton of ground ore of a water-soluble half ester salt of the above specified type, either with or without the addition of other collecting, frothing or conditioning agents or oils, and subjected to agitation and aeration in one of the well-known types of flotation cells. The operation of the process will be understood by a consideration of the following examples, it being understood that the invention is by no means limited to the conditions as outlined in the examples.

## Example 1

A sample of monoabietyl phthalate



was prepared by reacting equimolecular proportions of abietyl alcohol and phthalic anhydride in the manner described in an application of Barrett and Lazier Serial Number 749,070, filed October 19, 1934. Two grams (0.0046 mol.) of the monoabietyl phthalate was dissolved with the aid of gentle warming in 20 cc. of one per cent sodium hydroxide solution. After diluting to 100 cc., the resulting solution contained 0.0210 g. of the sodium salt of monoabietyl phthalate per cubic centimeter of solution and a very slight excess of sodium hydroxide.

Fifty pounds of bituminous slack coal was ground through a pulverizer of the horizontal disc type until all was finer than 40-mesh. The ground coal was thoroughly mixed and carefully sampled. A sieve analysis showed the following range of particle sizes.

| Size           | Weight percent |
|----------------|----------------|
| Plus 40-mesh   | 0              |
| Plus 60-mesh   | 56.5           |
| Plus 100-mesh  | 14.0           |
| Minus 100-mesh | 29.5           |
|                | 35             |
|                | 100.0          |

The crushed coal contained about 10 per cent of ash and 3 per cent of moisture.

One thousand grams of the ground coal was slurried with water and transferred to a laboratory flotation cell of the subaeration type. After adding water to fill the cell to the pulp level, 30 cc. of the solution of sodium monoabietyl phthalate was added. A froth loaded with coal particles quickly formed and flowed over the lip of the cell into a receiving vessel. The froth broke down rapidly allowing the coal particles to settle to the bottom of the receiving vessel. After 15 minutes at an agitator speed of 1100-1500 R. P. M., the collection of the first concentrate was finished. Another 5 cc. portion of the sodium monoabietyl phthalate solution was then added and a second concentrate of poorer qual-

- ity was obtained. During collection of this second concentrate the froth was again very satisfactory in volume and the floating coal was removed from the cell without any difficulty. The products were filtered, dried, and analyzed for their ash content with results as shown in the following table.

| 10 | Product            | Weight grams | Ash percent | Weight ash grams | Weight coal grams | Recovery percent |
|----|--------------------|--------------|-------------|------------------|-------------------|------------------|
|    | First concentrate  | 625          | 7.47        | 46.69            | 578               | 66.8             |
|    | Second concentrate | 265          | 10.51       | 27.85            | 237               | 27.4             |
| 15 | Tailings           | 78           | 36.17       | 28.21            | 50                |                  |
|    |                    | 968          | —           | 102.75           | 865               | 94.2             |

16 Ash in feed, dry basis, 10.62 per cent.  
 Total recovery of coal, 94.2 per cent.  
 Reagent: for first concentrate, 1.30 lbs. per ton.  
 20 for second concentrate, 0.22 lb. per ton.

### Example 2

25 A sample of an argillaceous limestone commonly known as "cement rock" was obtained from the quarry of the Valley Forge Cement Company, West Conshohocken, Pennsylvania. The rock was crushed in a small jaw crusher and then reduced to minus 40-mesh by means of a Braun disc pulverizer. After thorough mixing, 1000 g. of the ground rock was further pulverized by grinding for 75 minutes in a one gallon pebble mill with one liter of water and 3 kg. of flint pebbles. The ground slurry, now about 35 per cent minus 200-mesh, was split into eight approximately equal portions by means of a sample splitter.

30 A solution of the sodium salt of monoabietyl phthalate was prepared by dissolving 0.250 g. of monoabietyl phthalate in 46 cc. of 0.1 per cent sodium hydroxide solution and diluting to 100 cc. The resulting solution contained 0.00262 g. of sodium monoabietyl phthalate per cubic centimeter.

35 One of the portions of finely ground ore slurry was washed into a small laboratory flotation cell of the mechanical agitation type described by Gates and Jacobsen (Engineering and Mining Journal 119, 19, 771 (1925)). Ten cubic centimeters of the sodium monoabietyl phthalate solution was added and the agitator started. A froth well loaded with calcium carbonate particles was quickly produced without addition of any other reagent. After running for four minutes, collection of the first concentrate was completed. An additional 5 cc. portion of the reagent solution was added and a second concentrate was lifted into the froth. This second concentrate, also high in calcium carbonate, was collected in a separate container. After the run was completed the products were filtered, dried, weighed and analyzed for calcium carbonate, the results being shown in the following table.

| 5  | Product            | Weight grams | CaCO <sub>3</sub> percent | Weight CaCO <sub>3</sub> grams | CaCO <sub>3</sub> recovery percent |
|----|--------------------|--------------|---------------------------|--------------------------------|------------------------------------|
|    | First concentrate  | 40.2         | 90.2                      | 36.3                           | 39.5                               |
|    | Second concentrate | 39.0         | 95.8                      | 37.3                           | 40.7                               |
| 10 | Tailings           | 42.2         | 43.2                      | 18.2                           |                                    |
|    |                    | 121.4        | —                         | 91.8                           | —                                  |

15 Calcium carbonate in feed, 75.6% (calcd.).  
 Total recovery, 80.2%.  
 Reagent: for first concentrate: 0.43 lb. per ton.  
 for second concentrate: 0.215 lb. per ton.

### Example 3

20 A solution of the sodium salt of monododecyl phthalate was prepared by dissolving 0.250 g. of monododecyl phthalate in 34.5 cc. of 0.1 per cent sodium hydroxide solution and diluting to 100 cc. The resulting solution contained 0.00279 g. of sodium monododecyl phthalate and a small amount of free sodium hydroxide per cubic centimeter of solution. Another charge of ground cement rock similar to that used in the preceding example was placed in the small flotation cell, water added to fill the cell to the pulp level, the agitator started, and then 15 cc. of the sodium monododecyl phthalate solution added. A froth 25 of good volume and well loaded with calcium carbonate particles was produced. Flotation was complete in about 11 minutes and no further reagent additions were required. The products were filtered, dried and analyzed with the following results:

| Product     | Weight grams | CaCO <sub>3</sub> percent | Weight CaCO <sub>3</sub> grams | CaCO <sub>3</sub> recovery percent |
|-------------|--------------|---------------------------|--------------------------------|------------------------------------|
| Concentrate | 99.7         | 89.06                     | 88.8                           | 92.9                               |
| Tailings    | 28.9         | 23.46                     | 6.8                            |                                    |
|             | 128.6        | —                         | 95.6                           | —                                  |

30 Calcium carbonate in feed (calcd.), 74.32%.  
 Reagent used, 0.65 lb. per ton of feed.

### Example 4

35 A solution containing 0.0027 g. of sodium mono-n-octyl phthalate per cubic centimeter was prepared by dissolving 0.250 g. of mono-n-octyl phthalate in 45 cc. of 0.1 per cent sodium hydroxide solution and diluting to 100 cc. Ten cubic centimeters of this solution were used as the flotation agent in a test using a charge of ground cement rock as in the two preceding examples. A 40 satisfactory froth well loaded with calcium carbonate was produced. The flotation was complete in 7 minutes yielding results as summarized in the following table.

| Product     | Weight gram | CaCO <sub>3</sub> percent | Wt. CaCO <sub>3</sub> gram | CaCO <sub>3</sub> recovery percent |
|-------------|-------------|---------------------------|----------------------------|------------------------------------|
| Concentrate | 76.9        | 91.89                     | 70.66                      | 77.2                               |
| Tailings    | 45.1        | 45.17                     | 20.84                      |                                    |
|             | 123.0       | —                         | 91.50                      | —                                  |

55 Calcium carbonate in feed (calcd.), 74.39 per cent.  
 Reagent used, 0.44 lb. per ton.

60 A higher recovery could readily have been produced by the use of a slightly greater amount of the flotation reagent.

65 With certain types of ores, particularly those which are earthy and poorly crystalline in nature, it is frequently beneficial to employ a "collecting oil" such as crude petroleum oil, a coal tar or wood tar distillate, kerosene, Diesel oil, or the like, along with a frothing agent to effect the flotation of a desired mineral. As an example of a flotation carried out in this manner, the concentration of an earthy manganese ore by use of gas oil and fish oil soap as carried out by the Cuban Mining Company at Cristo, Cuba, may be cited. Sometimes it is distinctly beneficial to emulsify the oil in water before adding it to the ore pulp in order to produce better contact between the desired mineral and the oil. The reagents forming the subject of the present invention may be used very 70 75

## Example 6

An emulsion of the following composition was prepared:

|                                  |       |       |   |
|----------------------------------|-------|-------|---|
| Mono-octadecyl phthalate         | grams | 0.100 | 5 |
| Sodium oleyl sulfate (27% paste) | do    | 0.066 |   |
| Sodium hydroxide                 | do    | 0.150 |   |
| Coal tar oil                     | do    | 3.750 |   |
| Water, to make a total of        | cc    | 150   |   |

The coal tar oil used is an oil obtained in a low-temperature coking process. When distilled under atmospheric pressure, about 84 per cent of the oil distilled over in the temperature range of from 185° to 300° C., the remainder being a higher boiling residue. The oil contains cresols, xyleneols, and other phenolic, neutral, and basic ingredients.

A flotation test similar to that described in Example 5 was carried out using 46.5 cc. of the above emulsion. As before, a small amount of the oxygenated frothing oil boiling at 150-160° C. was added. Flotation proceeded satisfactorily giving a concentrate rich in the black manganese minerals. The concentrate weighed 37.6 g. or 57.5 per cent of the weight of the flotation feed. The quantities of reagents used were as follows:

|                                         | Grams | Pounds per ton |
|-----------------------------------------|-------|----------------|
| Mono-octadecyl phthalate                | 0.066 | 0.93           |
| Sodium oleyl sulfate (27% paste)        | 0.300 | 0.61           |
| Coal tar oil                            | 34.9  | 30             |
| Sodium hydroxide                        | 1.41  |                |
| Oxygenated frothing oil, B. P. 150-160° | 1.56  |                |

It has been found that a very great variety of water-soluble salts of half esters of organic dibasic acids may be used in ore flotation with very satisfactory results if the alcohol, with which one of the carboxyl groups of the dibasic acid is esterified, is chosen from the group comprising straight chain primary alcohols having from 8 to 18 carbon atoms and the alicyclic alcohols. The new class of flotation reagents may be represented by the following general formula:



In this formula, M represents an alkali metal such as sodium or potassium or an ammonium group; R, a divalent aliphatic, alicyclic or aromatic radical; and R', a long straight chain aliphatic radical having 8 to 18 carbon atoms in a saturated or unsaturated chain, or an alicyclic radical formed in the carboxylic reduction of a naphthenic acid or natural resin acid. Further, without departing from the scope of the present invention, the divalent radical, R, may possess various types of substituent groups such as hydroxyl groups, alkyl groups, unsaturated linkages, halogen groups, etc., or in a limiting case the radical, R, may be omitted altogether and the carboxyl groups joined directly to each other as in the case of oxalic acid.

The following are examples of suitable dibasic acids from which flotation agents coming under the scope of the present invention may be prepared:

Oxalic acid, succinic acid, adipic acid, sebacic acid, maleic acid, fumaric acid, malic acid, tartric acid, phthalic acid, tere-phthalic acid, hexahydrophthalic acid.

Alcohols with which one of the carboxyl groups of acids, such as the above, may be esterified are very numerous. The following partial list is illustrative of suitable alcohols which may be used in preparing the flotation reagents:

advantageously in ore flotation processes involving the use of emulsified oils, since they have been found to possess strong emulsifying power. Their emulsifying power, combined with their frothing and collecting properties as already illustrated, makes them extremely valuable reagents for use in the oil emulsion type of flotation process. Two examples of the use of the new type of flotation reagents in the oil emulsion flotation process follow.

## Example 5

One kilogram of minus 40-mesh manganese oxide ore from the Cuban Mining Company, Cristo, Cuba, was ground for 30 minutes in a one-gallon pebble mill with 3 kg. of flint pebbles, 1 liter of water and 5 g. of 40 per cent water glass. The ground charge was diluted to a volume of 4 liters and then run through a laboratory elutriator to separate the sandy portions of the ore from the nearly colloidal slimes. The settling, now largely free from slime, were slurried up with water and split into eight approximately equal samples for use in the small flotation cell described above.

An emulsion having the following composition was then prepared:

|                                  | Grams |
|----------------------------------|-------|
| Sodium oleyl sulfate (27% paste) | 0.066 |
| Monododecyl phthalate            | 0.300 |
| Sodium hydroxide                 | 0.300 |
| Panuco crude oil                 | 3.75  |
| Water                            | 50.00 |

The emulsion was diluted to a volume of 125 cc. prior to use. Panuco crude oil is a Mexican petroleum oil.

One of the deslimed ore charges was partially freed from water by siphoning off the supernatant water, and 38 cc. of the oil emulsion added. The mixture of ore slurry and emulsion was agitated for 90 seconds using a high speed drink mixer to afford thorough mixing and was then washed into the small flotation cell. As an aid to frothing, 2 drops (0.017 g.) of an oxygenated organic compound boiling from 150-160° C. prepared as described in the U. S. Patent of Charles L. Burdick, No. 1,995,915, was added. A very satisfactory froth carrying a heavy load of black manganese minerals was formed. The froth broke down rapidly in the receiving vessel indicating that in large scale practice the flotation concentrate could be sent to a thickener, for example, of the well-known Dorr type, to separate the mineral concentrate from the accompanying water. The products from the flotation test were filtered and dried. The concentrate was nearly black in color indicating it to be high in manganese oxides while the tailings were grayish brown and sandy in appearance, obviously nearly free of manganese.

The results may be summarized as follows:

| Product     | Weight gram | Weight percent |
|-------------|-------------|----------------|
| Concentrate | 43.8        | 54.3           |
| Tailings    | 36.8        | 45.7           |
|             | 80.6        | 100.0          |

Reagents used (lb. per ton of feed):

|                                  |      |
|----------------------------------|------|
| Monododecyl phthalate            | 2.26 |
| Sodium oleyl sulfate (27% paste) | 0.50 |
| Panuco crude oil                 | 28.3 |
| Sodium hydroxide                 | 2.26 |
| Frothing oil, B. P. 150-160°     | 0.42 |

n-octyl alcohol, n-decyl alcohol, n-dodecyl alcohol, n-tetradecyl alcohol, n-octadecyl alcohol, cetyl alcohol, oleyl alcohol, abietyl alcohol, dihydroabietyl alcohol, naphthenyl alcohols formed by carboxylic acid reduction of naphthenic acids from petroleum.

The preparation of many of the above mentioned half esters is described in more detail in Graves and Lawson Patents 1,993,736, 1,993,737, 10 and 1,993,738; in Barrett and Lazier Patent 2,047,664, and in a co-pending application of Barrett and Lazier, Serial No. 749,070, filed October 19, 1934.

The half esters formed by reaction of alcohols 15 and acids chosen from the above examples or similar half esters formed by any other suitable reaction are substantially insoluble in water, but, since they retain one free carboxyl group, they may be converted to water-soluble salts by neutralization with suitable bases such as sodium 20 hydroxide, potassium hydroxide, ammonium hydroxide, etc.

It will be evident that a very great number of 25 different half ester salts may be used in the operation of this invention without departing from the spirit thereof. As examples of specific reagents which are useful in carrying out the process, the following may be mentioned.

Sodium monododecyl phthalate, sodium mono- 30 abietyl phthalate, sodium mono-octadecyl phthalate, potassium monodihydroabietyl succinate, sodium mono-oleyl maleate, ammonium monododecyl phthalate, sodium mono-octyl succinate, sodium monodihydroabietyl phthalate.

35 By a proper choice of alcohol, dibasic acid and salt-forming base, it is possible to exert a very large degree of control over the collecting, frothing, and selective properties of this new type of flotation reagents.

40 The advantages of the invention derive largely from the fact that according to the teachings of this invention it is possible to exercise a very great degree of control over the frothing and collecting power of the reagents by suitable changes 45 in the molecular architecture. The reagents having very long carbon chains, say from 16 to 18 carbon atoms, are in general very powerful collecting agents and have great emulsifying power. The members having fewer than 16 carbon atoms 50 in the long chain in general may be said to have superior frothing power while largely retaining the collecting and emulsifying power of the higher members. When used in coal flotation, reagents of the class described in this invention give froths 55 which are not only well loaded with coal particles but which also build up to a sufficient volume that their removal from the cell is greatly facilitated. Further, the froths break down rapidly in receiving vessels to a mixture of coal and water 60 from which most of the water may be drained off readily. This is not true of the older coal flotation reagents such as kerosene, cresylic acid and pine oil, which give very stable froths which are difficult to dewater. A further advantage is 65 that the new reagents frequently give satisfactory results when used in considerably smaller amounts than is possible with those previously known.

In carrying out the processes of the present 70 invention many modifications which may be made without departing from the spirit of the invention will be evident to those versed in the art of ore flotation. Thus, for example, any of the well-known types of flotation cells may be used. The 75 ratio of solids to water in the ore pulp may vary

from about 1:1 to 1:6. The reagents may be used alone, since most of them have strong frothing power as well as collecting power, or they may be used in conjunction with previously known collecting, frothing, and conditioning agents. 5 Since the reagents have the power to emulsify oils, they are very useful in the flotation process which employs oils emulsified in water prior to addition to the pulp. It is usually preferable to work in a neutral or alkaline pulp since the reagents are precipitated from solution by mineral acids. The salts employed may be added before, during or after grinding or during the course of the flotation operation itself. Sometimes mixtures of two or more of the reagents of the 15 present invention may be used together to ad-

These reagents are particularly adapted for use in the flotation of non-sulfide minerals of the type having an alkaline earth metal in the positive portion of the molecule, for example, calcite, fluorspar, barite, apatite, witherite, magnesite, dolomite, etc. They are not well adapted to the flotation of quartz and the silicate minerals, and, for this reason, good separation of 20 the named alkaline earth minerals are possible. They are also useful in the flotation of carbonate minerals of the heavy metals, such as rhodochrosite, smithsonite and cerussite. When used as a component of an oil emulsion, they are excellent reagents in the flotation of oxide ores of manganese. They have been found to be excellent reagents for use in coal flotation. 30

The above description and examples are to be taken as illustrative only and not as limiting the 35 scope of the invention. Any variation or departure therefrom which conforms to the spirit of the invention is intended to be included within the scope of the appended claims.

We claim:

1. In the froth flotation process of treating ores, the step which comprises utilizing as a flotation agent a water-soluble salt of an organic dicarboxylic acid having one carboxyl group esterified by an alcohol selected from the group 45 consisting of long chain primary aliphatic alcohols having from eight to eighteen carbon atoms and alicyclic alcohols formed in the carboxylic reduction of a naphthenic acid or a natural resin acid. 50

2. In the froth flotation process of treating non-sulfide ores and coal, the step which comprises utilizing as a flotation agent a water-soluble salt of an organic dicarboxylic acid having one carboxyl group esterified by an alcohol 55 selected from the group consisting of long chain primary aliphatic alcohols having from eight to eighteen carbon atoms and alicyclic alcohols formed in the carboxylic reduction of a naphthenic acid or a natural resin acid. 60

3. In the froth flotation process of treating non-sulfide ores and coal, the step which comprises utilizing as a flotation agent an alkali metal salt of an organic dicarboxylic acid having one carboxyl group esterified by an alcohol 65 chosen from the class consisting of straight chain aliphatic primary alcohols having from eight to eighteen carbon atoms and alicyclic alcohols formed in the carboxylic reduction of a naphthenic acid or a natural resin acid. 70

4. In the froth flotation process of treating non-sulfide ores and coal, the step which comprises utilizing as a flotation agent a water-soluble salt of an aromatic dicarboxylic acid having one of the carboxyl groups esterified with 75

an alcohol chosen from the class consisting of straight chain aliphatic primary alcohols having from eight to eighteen carbon atoms and alicyclic alcohols formed in the carboxylic reduction of a naphthenic acid or a natural resin acid.

5. In the froth flotation process of treating non-sulfide ores and coal, the step which comprises utilizing as a flotation agent an alkali metal salt of an aromatic dicarboxylic acid having one of the carboxyl groups esterified with an alcohol chosen from the class consisting of straight chain aliphatic primary alcohols having from eight to eighteen carbon atoms and alicyclic alcohols formed in the carboxylic reduction of a naphthenic acid or a natural resin acid.

6. In the froth flotation process of treating non-sulfide ores and coal, the step which comprises utilizing as a flotation agent an alkali metal salt of an ester of phthalic acid having one of the carboxyl groups esterified with an alcohol chosen from the class consisting of straight chain aliphatic primary alcohols having from eight to eighteen carbon atoms and alicyclic alcohols formed in the carboxylic reduction of a naphthenic acid or a natural resin acid.

7. In the froth flotation process of treating non-sulfide ores and coal, the step which comprises utilizing sodium mono-abietyl phthalate as a flotation agent.

8. In the froth flotation process of treating cement rock, the step which comprises utilizing as a flotation agent an alkali metal salt of an ester of phthalic acid having one of the carboxyl groups esterified with a straight chain aliphatic primary alcohol having from eight to eighteen 10 carbon atoms.

9. In the froth flotation process of treating manganese oxide ore, the step which comprises utilizing as a flotation agent an oil-in-water emulsion containing an alkali metal salt of an 15 ester of phthalic acid having one of the carboxyl groups esterified with a straight chain aliphatic primary alcohol having from eight to eighteen carbon atoms.

10. In the froth flotation process of treating non-sulfide ores and coal, the step which comprises utilizing sodium monododecyl phthalate as a flotation agent.

20

25 JAMES EMORY KIRBY.  
JAMES HERBERT WERNITZ.